

April 2, 1940.

J. O. BETTERTON ET AL

2,195,809

CONTINUOUS CASTING

Filed June 22, 1936

2 Sheets-Sheet 1



INVENTORS  
Jesse O. Betterton  
By Frank T. Poland  
James K. Fenix  
ATTORNEY

April 2, 1940.

J. O. BETTERTON ET AL

2,195,809

CONTINUOUS CASTING

Filed June 22, 1936

2 Sheets-Sheet 2

Fig. 2



Fig. 3



Fig. 5



Fig. 4



INVENTORS  
Jesse O. Betterton  
BY Frank F. Poland  
James K. Kent  
ATTORNEY

## UNITED STATES PATENT OFFICE

2,195,809

## CONTINUOUS CASTING

Jesse O. Betterton, Metuchen, and Frank F. Poland, Highland Park, N. J., assignors to American Smelting and Refining Company, New York, N. Y., a corporation of New Jersey

Application June 22, 1936, Serial No. 86,600

12 Claims. (Cl. 22—200.1)

This invention relates to the art of continuous casting of non-ferrous metals, particularly copper and copper alloys, and provides certain improvements in that art whereby metal shapes 5 of indefinite length may be produced on a commercial scale in a truly continuous manner. While the invention will be described with reference to the continuous casting of copper or copper alloys, it will be understood that the 10 principles thereof are, for the most part, applicable to the casting of other non-ferrous metals and alloys which present problems similar to those encountered in continuously casting copper or its alloys.

15 The concept of continuously casting non-ferrous metals such as copper and copper alloys, that is, by supplying the molten metal from a reservoir to one end of a die or mold having solid metal in the other end which serves as a 20 plug and to which the molten metal welds as it solidifies accompanied by withdrawal of the cast shape at a rate substantially equal to that 25 of solidification, is indeed an old one and various and sundry processes and apparatus have been proposed for its fulfillment.

However, when it is attempted to pursue these prior art teachings in practice one immediately finds them fraught with difficulties and obstacles for the satisfactory solution of which one searches 30 their sponsors' teachings in vain. Chief among these difficulties and obstacles are: physical unsoundness of the cast metal both internally (piping, gas pockets, and other defects caused by accumulation or entrapment of gas) and externally (cracked, checked or otherwise defective surface); breakage of the cast shape resulting in losses due to the breakage itself and otherwise highly undesirable because of damage to the apparatus and exposure of the workmen to 35 danger by reason of runouts of the molten metal which all too frequently accompany breakage of the casting; and the inability or failure of such proposals, insofar as any of them do produce any sound metal, to do so as a truly continuous and satisfactory commercial operation.

Generally speaking, investigation has shown that the inability of the prior art processes and apparatus to produce sound castings in a truly continuous manner and on a satisfactory commercial scale may be attributed, either directly or indirectly, to two things: entrapment of gas in the solidified metal and friction between the die or mold and the metal. The present invention by providing a modus operandi which 45 eliminates the former and minimizes the latter,

effectively solves the problem thereby permitting copper and copper alloy shapes of indefinite length to be continuously cast at rates which are definitely commercial.

Investigations and experiments have clearly 5 indicated and demonstrated that mold friction and gas entrapment can be overcome or controlled to the extent prerequisite for successful continuous casting if certain factors or conditions are fully appreciated and observed. That 10 some of these factors or conditions are more or less independent while others are closely interrelated with other factors with respect to the manner in which the several factors, by their proper observance, contribute to the desired result, will be apparent as the description proceeds. These factors and conditions, the importance and correct observation of which have been amply and repeatedly confirmed in actual practice, may 15 be summarized as follows:

20 1. Proper preliminary preparation of the copper or copper alloy.

2. Introduction of the molten metal into the mold in a manner avoiding turbulence of the metal therein.

25 3. Avoidance of a deep head of molten metal on that in the mold.

4. Provision of a mold of proper design in which at least the inner surface thereof that contacts the molten and freshly solidified copper 30 complies with certain requirements.

5. Proper control of the "intermediate" zone which is hereinafter defined and described.

Before entering into the detailed discussion and explanation of the several factors enumerated above, it may be said that continuous casting processes may be roughly classified with respect to the manner or method by which at least the major portion of the heat is withdrawn from the molten metal to effect its solidification as: (a) lateral cooling, that is, by extraction of the heat through the mold wall and (b) longitudinal cooling, that is, by extraction of the heat through the previously solidified copper. Naturally there may be said to be a third 40 class in which substantial heat extraction is accomplished both laterally and longitudinally. However, this is really a matter of degree, since, as a practical matter, there is always at least some small amount of heat extracted longitudinally in any lateral cooling process and vice versa. Accordingly, it seems better for the sake of clarity to classify all the processes as (a) or (b) according to whether a major portion of the heat (50% or more) is extracted laterally 45 50 55

or longitudinally in effecting solidification of the copper. For reasons that will become apparent as the description proceeds, the present invention contemplates a process in which lateral 5 cooling is employed although observance of many of the factors yields improved results in longitudinal cooling processes as well.

For a better understanding of the invention and the roles played by the several factors mentioned, it may be pointed out that all commercial processes for casting copper must deal with metal containing gases, it being well known and generally acknowledged in the art that liquid copper in contact with a gaseous atmosphere will have 10 some gas dissolved or occluded therein. In addition, the tensile strength of copper at temperatures approaching its melting point is very low and hence copper just as it solidifies is extremely 15 fragile. Further, the surface tension of molten 20 copper is low.

Turning now to the various factors already set forth and which are listed without regard to order of importance, the first to be considered is the preliminary preparation of the copper 25 which consists essentially in rendering it substantially gas-free, oxygen-free prior to its introduction into the mold.

It will be remembered that the continuous casting process contemplates continuously leading 30 the molten copper from a supply thereof into one end of a suitable mold, the other end of which is closed by previously solidified copper, and causing the molten copper so introduced to solidify and weld to the previously solidified 35 copper, the resulting cast shape of indefinite length being continuously withdrawn from the mold. In other words, the molten copper is formed into a moving column and as one end thereof is solidified and continuously withdrawn, 40 the other end of the moving column is replenished with molten copper.

Now as the copper solidifies, the gases dissolved 45 therein are liberated from the freezing copper and pass into the intermediate zone (hereinafter treated in detail) so that it might seem, at first glance, that castings closely approaching pure copper in density could be continuously produced merely by freezing the metal from the bottom 50 upward. Unfortunately for the art, the problem is not so simply solved if casting speeds sufficiently high to place the operation on a satisfactory 55 commercial plane are to be continuously maintained. Oft repeated runs have conclusively demonstrated that failure to effect a substantial degasification of the copper prior to its introduction into the mold invariably invites breakage of the casting with its attendant losses as well as unsoundness in whatever cast shape is obtained.

60 The contribution which prior degasification of the copper makes to the success of the continuous casting operation is no doubt due in a large measure to the fact that the liberation of the gases occurs at the freezing line of the metal in the mold which is the very place where the newly 65 solidified copper exhibits its maximum degree of fragility. Hence, the clear indication is that the less gas there is liberated at this delicate zone, the less chance for gas entrapment or for stresses 70 and strains to be set up incident to gas movement. Further, deoxidation of the copper prevents oxidation and consequent roughening of the interior or the inner surface of the mold, which as hereinafter shown is of carbon, thus 75 reducing mold friction and minimizing surface

imperfections in the casting which otherwise would result from the roughened surface.

The treatment of the copper preparatory to introducing it into the mold may be effected in accordance with usual refining practise by first 5 blowing it with air until the hydrogen and sulphur are expelled as completely as possible and then poling the resulting low set copper to a point where cast samples will have a density of at least 8.50. The resulting copper, though commercially gas-free, still contains a small amount 10 of oxygen (less than 0.01%) and this is removed in any suitable manner as by incorporating small but sufficient amounts of a metallic deoxidizer 15 therein. Phosphorus is an efficient deoxidizer and if used is preferably employed in a manner 20 which imparts to the copper an approximate residual phosphorus content of from 0.001% to 0.005%. The copper so prepared being substantially gas-free, oxygen-free is now suitable for 25 introduction into the mold. It will, of course, be understood that if it is desired to cast copper alloys instead of copper, the necessary alloy constituents for the particular alloy desired may be incorporated in the prepared copper prior to introducing the metal into the mold.

The second factor enumerated above is that of introducing the molten copper into the mold in such manner that turbulence of the metal therein is avoided. This factor is closely related to 30 the extremely fragile nature of the freshly cast or newly solidified copper, it having been found that breakage of the newly cast shape is greatly aggravated when copper is introduced in a manner imparting turbulence to the metal in the 35 mold.

While various methods and means will, no doubt, occur to those skilled in the art for maintaining the metal in the mold in a quiescent state, one manner of introduction that has 40 proved entirely satisfactory in actual practise is to introduce the prepared molten copper into the receptacle or reservoir in which the mold is mounted at a point sufficiently remote from the mold that turbulence of the metal incident to its 45 introduction into the reservoir will have subsided before the mold entrance is reached.

Failure to observe this factor in introducing the molten copper is to invite breakage of the casting and consequent interruption of the continuity of the process. Furthermore, cessations 50 in operation occasioned by breakage of the casting are, of course, of a much more serious nature than a simple discontinuance of the casting process but even to practise the latter to avoid breakage when adding copper to the receptacle 55 would mean loss or delay each time in the subsequent starting up period as will hereinafter be apparent.

The third factor to be considered is that of 60 avoiding a deep head of metal on that in the mold, which factor is probably closely related to both the low surface tension of the molten copper and the low tensile strength or fragility of the newly solidified copper.

65 It has been observed that whenever a deep head of metal is present above the copper undergoing solidification in the mold, there is a marked tendency of the casting to emerge from the mold with a rough, checked or cracked surface and 70 even to break entirely in two.

Considering the fragile nature of the freshly solidified copper and the low surface tension of the molten copper, the explanation of the checked or cracked surface may be that the hy- 75

drostatic pressure exerted by the head of metal above the mold causes the molten and solidifying copper therein to spread out and that with an excessive head of molten copper above the mold 5 for the diameter of the particular casting there is produced such a degree of friction between the mold and metal as to cause a slipping between the crystals of the copper before same are thoroughly set through complete freezing. However, the exact cause or explanation of such 10 defects is immaterial, it being a fact that whenever the depth or head of molten copper becomes excessive for the diameter of the rod being cast, the imperfections hereinbefore noted result.

15 The working range of the depth or head of metal may be said to vary from such depth as will fill the mold without turbulence, as the minimum, to such depth as will just fail to produce the imperfections noted, as the maximum. A 20 safe working rule is to maintain the head of molten copper above the mold between the approximate limits of one inch minimum to six inches maximum as same has been found in practise to fulfill the requirements for any diameter casting produced by the continuous process.

25 The fourth factor concerns the provision of a suitable mold, experience having shown that for at least that surface of the mold which contacts the copper in the vicinity where solidification of 30 the copper is effected, particular care must be exercised both in the selection of the material therefor and in the preparation of same.

Because of the low surface tension of molten copper, it tends to flow into any surface imperfections such as cracks, pores or other irregularities in the interior mold wall and by solidifying therein to produce fins or other irregularities in the casting which, by reason of the increased friction between the copper and the mold, lead 40 to fracture of the casting. It should be mentioned in this connection that friction between the mold wall and the newly solidified copper must be maintained at the lowest feasible minimum or failures in the process will inevitably result by reason of the low tensile strength of 45 the newly solidified copper.

In view of what has just been said it will be clear that the interior surface of the mold which contacts the molten and newly solidified copper 50 should be as mechanically perfect as it is possible to produce and of a material which does not react with copper to any extent. For a lateral cooling process, such as is contemplated by the invention, it has also been definitely established that the mold should be as thin-walled as possible 55 and of a material possessing at least a reasonable degree of heat conductivity.

Actual practise has shown that commercial and sustained casting operations may be accomplished 60 through the use of a mold of dense graphite having a particle size not exceeding 40 microns as the maximum and of a porosity of not more than 20% with pore spaces of 40 microns maximum. Such a grade of graphite, which may be produced by chemical precipitation and cementation under high pressure employing colloidal carbon as the bond, is not to be confused with other grades which are commonly referred to as dense graphite but which do not meet the above specifications.

70 The last of the factors listed is that of proper control of the intermediate zone and as the description proceeds it will be apparent that a thorough understanding of same and intelligent manipulation thereof are invaluable in obtaining

commercial results particularly in a process such as that of the invention which employs lateral cooling.

In continuously casting copper, the molten copper must, of course, be cooled from the liquid 5 to the solid phase. The initial cooling extracts the superheat from the metal thus reducing its temperature to the melting point and further cooling, by extracting its latent heat of fusion, converts the liquid copper at its melting point 10 into solid copper at the same temperature. Between the fully molten phase of the copper and its solid phase there is, therefore, a region in which the latent heat of fusion of the copper is being extracted and in which the actual freezing 15 of the copper is taking place. This region, for want of any better descriptive term, is referred to herein as the intermediate zone and the extent of the intermediate zone, that is, the distance between two parallel planes defining same (one 20 plane wholly in the molten phase and the other wholly in the solid phase) is referred to in the present description and appended claims as the "depth" of said zone.

While experts may perhaps differ as to the 25 actual physical condition of the copper in this intermediate zone, same is not of importance in view of actually observed results which show the intermediate zone to be the zone of gas entrapment. Numerous specimens of cast copper prove 30 conclusively that as the metal freezes, the gases dissolved therein are liberated incident to the solidification of the metal and pass into the intermediate zone. If the intermediate zone is properly controlled as herein provided, sound 35 castings may be continuously produced at rates which are definitely commercial; if it is not so controlled failure ensues.

As hereinbefore indicated, the present invention contemplates lateral rather than longitudinal 40 cooling, that is, the extraction of heat from the copper in order to solidify same is accomplished laterally through the mold wall. This is significant because while it has long since been proposed, the obstacles which it presented to 45 commercial adaptation were apparently considered insuperable by those in the field as witnessed by the later advent into the casting art of the longitudinal cooling principle. Results obtained by the present invention, however, show that if the factors heretofore discussed are 50 observed and the intermediate zone regulated or controlled as next disclosed, sound copper castings can be continuously produced at commercial 55 rates materially above the inherently limited production of any known longitudinal cooling process.

It has been found that if the intermediate zone is at all times maintained such that the crystals of the cast copper are disposed radially, 60 that is, a structure in which the crystals are inclined in predominating numbers at an angle of 45° or more to the axis of the billet or rod, such inclination being upward from the circumference of the cast shaped toward the freezing 65 surface of the copper, sound castings can be continuously produced indefinitely, there being no entrapment of gases if the intermediate zone is so maintained as to produce such radial crystallization.

The production of only sound copper castings 70 through control of the intermediate zone to maintain radial crystallization whereby no gases become entrapped may perhaps be explained on the basis that in a lateral cooling process the 75

copper next adjacent the mold wall through which the heat is extracted will be the first to solidify while that nearest the center of the mold will be the last to solidify. This means, then, 5 (assuming a vertically disposed mold) that with lateral cooling the freezing line will be of a V-shaped nature as contrasted to a horizontal freezing line in a normal, longitudinal cooling process. From this it appears reasonable to 10 conclude that when entrapment of gases occurs it is because the inclination of the V-shaped freezing line is so steep that the gases passing into the copper in the intermediate zone as they are liberated from the freezing metal, cannot 15 escape before the copper in the intermediate zone is itself frozen. This view can be and is supported by actual observation inasmuch as the crystal structure of copper indicates the direction of heat flow during the freezing process. 20 Stated in a somewhat different manner, it has been definitely established that to insure the continuous production of a sound casting, the intermediate zone must be maintained below a maximum depth. While this maximum depth 25 may vary somewhat with different metals, it has been found that for copper, the intermediate zone must be restricted to a depth not greatly in excess of the diameter of the casting if entrapment of gas is to be avoided. It is, however, 30 a safe working rule for other non-ferrous metals or alloys because, even though the depth may be increased for some (e. g., those containing no gas or which can be completely degasified by preliminary treatment), it has been found in actually 35 casting various alloys that the operation can be continuously conducted at commercial speeds by employing the "diameter" rule.

The maintenance of a radial crystal structure, or control of the intermediate zone within a sufficiently shallow depth, has been found to be a 40 function of cooling or heat extraction and the process of the invention conclusively demonstrates that in order to obtain high casting speeds or rates which are so much desired, a 45 rapid cooling or solidification of the copper must be effected in order to maintain the proper intermediate zone. In fact, given proper observance of the other factors set forth, there is every indication that the only limitation, other 50 than die friction, upon the casting speed (rate of withdrawal of the casting from the mold) is that of the rate of heat extraction. In other words, the casting speed can be said to depend upon how quickly the heat from the molten copper 55 can be withdrawn through the mold wall and dissipated. The pertinency of the proper mold construction and provision for its vigorous cooling in this connection will, accordingly, be apparent.

60 A feature not heretofore separately discussed but which is closely related to the control of the intermediate zone and the successful conduct of the process, is the proper control of the casting speed. It is perhaps clear in view of what has already been said that the casting speed is dependent upon the rate of cooling and, hence, 65 must not be so great as to deepen the intermediate zone past its maximum depth. However, there are other facts worthy of specific mention 70 with regard to initiation of the operation. It has been found in practice that the full, commercial casting speed must be arrived at only by slow, gradual increments and without any sudden jerking of the casting being withdrawn and 75 that when the higher speed is once attained the

continuous withdrawal of the casting must be accomplished in a steady, uninterrupted manner. If this is not observed, breakage of the rod will result by reason of the low tensile strength of the newly solidified copper in the mold. 5

Further, in initiating the casting operation the rate of cooling must be adjusted with respect to the casting speed and the two correlated in order to attain the higher commercial speed desired. One of the most important reasons for this resides in the fact that if the full cooling rate is employed at such time when the casting speed is necessarily low, there is real danger of the copper freezing above the opening leading from the reservoir of copper into the mold thus 10 causing the casting to break as same continues to be withdrawn from the mold. On the other hand, if the intermediate zone is permitted to exceed its maximum depth through insufficient cooling, gas entrapment, attended by the production of unsound metal or breakage of the casting, will result. 15 20

While the novel features which are believed to be characteristic of this invention will be particularly pointed out in the claims appended 25 hereto, the invention itself and the manner in which it may be practised will be more readily understood by reference to the following description taken in connection with the accompanying drawings, in which 30

Fig. 1 represents, diagrammatically, a type of casting furnace and related assembly which may be employed in practising the invention, the view showing the casting furnace in longitudinal section; 35

Fig. 2 is an enlarged sectional elevation of the mold illustrated in Fig. 1, showing the details of the mounting of the mold in the casting furnace and the cooling arrangement therefor; 40

Fig. 3 is a view similar to that of Fig. 2 showing the cooling jacket for the mold in a lowered position; 45

Fig. 4 is a sectional plan view taken on the line 4-4 of Fig. 2;

Fig. 5 is a section elevation of a somewhat 45 different type of mold from that shown in Figs. 2 and 3.

Like reference characters denote like parts in the several figures of the drawings.

Referring to Fig. 1, 10 indicates generally a 50 casting or holding furnace having side walls, end walls 12 and 14, bottom 16 and roof 18 and an arch 20 extending transversely across the furnace near the charging end thereof. A charging port 22 is positioned in the roof 18 while burner opening 24 and flue 26 are provided in end walls 12 and 14, respectively. The bottom of the furnace and the side and end walls to a position above the metal line 28 of the furnace have a carbon lining 30. A charging spout or ladle 32 communicates with the interior of the furnace at its firing end while a normally closed tap hole (not shown) leads from the interior of the furnace to spout 34 at the flue end of the furnace. 55 60 65

The mold 36 in which the copper is continuously cast is mounted in an inverted cup-shaped holder 38 which in turn is positioned and secured in the floor of the furnace by suitable means, such as bricks 40 and refractory cement, at a point remote from that at which the molten metal is charged to the furnace 10. A variable screw 42 equipped with control wheel 44 is supported by brace 46 and connected to water jacket 48 for adjusting the latter with respect to the 70 75 80 85 90 95

mold 36. Adjustable grooved rolls 50 for withdrawing the cast billet or rod 52, die 54 and reel 56 are appropriately indicated.

Referring to the detail drawings, particularly Figs. 2 and 3, it will be seen that the mold 36, which is constructed from the special grade of dense graphite hereinbefore specified, is countersunk in and mounted flush with the top of the holder 38. A lock nut 58 secures the mold in the holder. Completely surrounding mold 36 is the relatively thick-walled water jacket 48 made from a metal of high heat conductivity such as forged copper and provided with water inlet 60 and outlet 62.

To insure a close fit between water jacket and mold when the former is in its uppermost position as shown in Fig. 2, as for normal full speed operation, but at the same time to provide for ready lowering of the jacket as shown in Fig. 3, as for less cooling when initiating the operation, both water jacket and the thin-walled portion of the mold are slightly tapered as indicated in the drawings thereby permitting them to be adjusted with respect to each other by raising or lowering the jacket by turning the screw 42.

Below the mold 36 and secured in place by any suitable means (not shown) is mold extension 64 shown as comprising two half sections 66, 68 yieldably joined by an ordinary bolt and spring arrangement as illustrated in Figs. 2 and 4. Each section of the mold extension is provided with a water inlet 70 and an outlet 72. The mold extension is appropriately of copper and has a graphite liner 74.

Fig. 5 shows a somewhat different type of mold 76 and water jacket 78, the former having a wider bore above the freezing zone than does the mold shown in Figs. 2 and 3 and the jacket is shown as tightly shrunk on the mold although it is obvious that the water jacket and mold may be made adjustable with respect to each other in the manner illustrated in Figs. 2 and 3. Otherwise the constructions are essentially the same. In all three figures, the intermediate zone is diagrammatically indicated by reference character 80, 52 being the solidified casting and 82 the fully liquid metal.

Employing apparatus such as just described, the invention may be practised as follows: the copper after being brought to the commercially gas-free state and deoxidized, which may be accomplished in the manner hereinbefore disclosed, is charged to the casting furnace or reservoir 10 via port 22 through the deep bed of carbon 84 which is preferably pre-ignited charcoal of low sulphur content as is also the layer 86. The copper in the furnace 10, which is kept in a fully liquid state by a burner (not shown) positioned in the opening 24, is maintained at a proper level, that is, one at which the head of metal above that in the mold 36 is not excessive, by appropriate additions from time to time. It is to be noted that turbulence of the copper in the mold 36 is avoided by positioning the mold in the floor of the furnace at a point remote from the charging end of the furnace. A plug extending upwardly into the mold and which is appropriately the last part of the casting from a previous run prevents the copper from being exited through the mold during the initial charging of the furnace before the casting operation is started.

In starting up, cooling water is circulated through the water jacket to solidify the copper 75 in the mold and weld it to the rod 52 which is

slowly withdrawn from the mold by rotation of the grooved rolls 50, it being understood that said rolls may be adjustable to each other for accommodating castings of different diameters and that either roll may be power driven in a known manner as by a variable speed motor coupled to a speed reducer and under a suitable rheostat control.

To bring the casting speed up to full commercial operation, the casting is steadily withdrawn at gradually increased rates simultaneously with increased cooling of the mold for the reasons heretofore explained. Different means may be employed for correlating the rates of cooling and withdrawal during this period. With a mold such as is shown in Fig. 5 where the water jacket is tightly shrunk on the mold, it is best accomplished by regulating the rate at which water is circulated through the jacket. In an assembly such as that shown in Figs. 2 and 3, it is preferably accomplished by starting the operation with the jacket in a lowered position as illustrated in Fig. 3 and gradually raising it into closer proximity to the mold wall as the rate of withdrawal of the casting increases until it at last snugly fits the mold wall and exerts its maximum cooling efficiency at which time the casting speed will be at full, commercial rate. One advantage of the adjustable water jacket is that the same vigorous flow of water can be maintained through it at all times as the rate of cooling is controlled by simply altering the space between jacket and mold as illustrated.

From the mold 36 in which the proper intermediate zone is maintained as before explained and the copper solidified, the casting is withdrawn through the mold extension 64, which being in sections, yieldably interconnected as shown, is self-adjusting to the rod produced by the particular sized bore of the mold being employed. Inasmuch as the formation of the casting is, and must necessarily be, performed in the mold 36 if sound copper castings are to be obtained, the water-cooled mold extension is not absolutely necessary. However, it is highly desirable as a safety precaution as it precludes run-outs in event of breakage of the casting and it also serves to prevent oxidation of the hot casting which would otherwise occur as it issues from the mold, the metal being and remaining bright as it emerges from the mold extension, thus dispensing with any necessity for pickling operations.

It may be here noted that while the mold 36, or at least the inner surface thereof in the case of a composite mold, is made from the special grade of dense graphite previously mentioned, ordinary grades of graphite may be used to line the mold extension as the copper has already passed through its molten and critically fragile state by the time it enters the mold extension. In this same connection it will be observed that as a matter of terminology the word "mold" is used to denote the apparatus in which the physical solidification of the copper is effected to clearly distinguish it from any similar structure in which this delicate operation is not performed such as the "mold extension" herein which does, however, cool the hot casting.

Passing from the mold extension and through the rolls 50, the casting 52 may be disposed of as desired in manners well known to the art. For example, it may be drawn through a die 54 or a series of dies and wound onto reel 56 or it may be severed by a suitable saw arrangement 75

into desired lengths as it emerges from the rolls 50 as may well be the case in casting, say, three inch billets.

It will be understood that various modifications and changes in the construction of equipment as well as variations in the details of operation thereof may be indulged in or practised without departing from the invention. Some are shown in the drawings and others will, of course, 10 occur to those skilled in the art. As to the former, it may be said that in constructing the mold shown in Figs. 2 and 3 it may be made with a straight bore except for a slight inward taper extending upwardly from the water jacket to 15 the mouth of the mold, this taper being approximately one quarter of an inch per foot. When heated to operating temperature, expansion reduces the taper so that the mold offers a substantially straight-walled bore to the copper 20 passing therethrough.

Fig. 5 illustrates a mold with an enlarged opening which in practise apparently offers some advantages in casting rod of small diameter by facilitating gas escape and minimizing agitation 25 of the copper in the intermediate zone incident to gas movement. On the other hand, due to the offset in such a mold immediately above the intermediate zone, greater care must be taken in correlating the rates of cooling and withdrawal 30 particularly when starting up to avoid "freezing" the apparatus.

Also while the mold wall should be as thin as possible to facilitate the high and rapid cooling rate demanded if the intermediate zone is to be 35 properly controlled at full commercial casting speeds, a much thicker graphite lining may be employed in the mold extension. Also instead of having one relatively long multiple-pieced or even one-pieced mold extension, two or more 40 shorter ones can be employed.

It may also be pointed out that in the particular type of mold mounting illustrated in the drawings, the sides of the holder 38 taper outwardly and downwardly which construction 45 makes for ease in dismounting same when this becomes necessary. Further, by reason of the mold being of graphite, it is well in practise to maintain a reducing atmosphere in the space within the holder where the mold is exposed to 50 prevent oxidation of same.

That copper can be continuously cast at commercial rates through the use of the invention has been amply demonstrated. For example, using a mold having a straight bore of one inch 55 and a mold wall only one quarter of an inch thick around which was shrunk a water jacket three inches long through which water was circulated at the rate of 70 pounds per minute, a casting speed of 20 inches per minute was easily 60 maintained with the production of sound, dense, one-inch diameter copper rod of a specific gravity exceeding that of rolled annealed copper, being over 8.93, the specimens of the rod so tested showing a specific gravity of at least 8.95. In a 65 somewhat similar run on copper-bronze, a casting speed of approximately 30 inches per minute was successfully maintained. As to the truly continuous nature of the process, little need be said further than that rod approximately half a 70 mile in length has been cast without a single break and that up to the point when the operation was finally voluntarily shut down, sound, dense rod was being continuously withdrawn. It may be mentioned that that particular run was 75 started on copper and finished on copper bronze,

the change being effected without interrupting the continuity of the casting process.

It has already been indicated that in addition to copper the principles of the invention are applicable to copper alloys and other nonferrous metals or alloys thereof, the continuous casting of which offers problems of a similar nature to those encountered in continuously casting pure copper. Among those which have already been successfully cast in accordance with the invention are: aluminum, copper-tin-tellurium, copper-silicon-tellurium, copper-nickel, copper-silicon, phosphor-copper, zinc-copper and aluminum-copper.

The castings produced in accordance with the present invention possess numerous advantages, many of which exist by reason of the radial crystal structure of the product. Thus, in rolling and annealing, the structure produced is one in which the crystals are random and equiaxed in orientation thereby producing in the product uniform forming qualities in all directions which is highly desirable in the production of articles with a rounded periphery. This is a definite advantage over a longitudinal crystal structure wherein the crystals are large and are oriented in a uniform plane and direction and retain such directional orientation even when rolled and annealed.

Of particular importance among the new results attainable by the process of the invention is the production of a new metallurgical product comprising copper and 0.001% to 0.005% phosphorus having a density of 8.93 or more (8.95 being common in practise) and possessing a radial crystal structure, that is, one in which the crystals are inclined in predominating numbers at an angle of at least 45° to the longitudinal axis of the casting; such product having been found to possess unexpected properties which render it markedly superior to any other copper product heretofore known for a host of uses. Such product can be readily cast in accordance with the invention, the proper phosphorus content being supplied when deoxidizing the copper prior to casting.

What is claimed is:

1. The process for casting non-ferrous metals and alloys which comprises degasifying same, maintaining the metal in its degasified state and confining it as a moving column, applying lateral cooling to the column such that, at the rate of casting employed, the intermediate zone is no greater than the minimum cross-sectional dimension of the column and radial crystallization of the metal as it solidifies is effected, and maintaining the metal in the column in a quiescent state by continuously feeding additional degasified metal thereto without turbulence.

2. The process for continuously casting copper and copper alloys which comprises refining same to render it commercially gas-free and deoxidized, establishing a moving column of the refined metal under substantially atmospheric pressure, withdrawing heat laterally from the moving column at such rate that the depth of the intermediate zone is less than the minimum cross-sectional dimension of the column and the metal solidifies with a radial crystal structure, and replenishing the supply of refined metal without turbulence to the moving column of metal.

3. In a continuous casting process for non-ferrous metals and alloys in which solidification of the metal is effected by laterally cooling a moving, vertical column thereof, said column being in open communication with a supply of

molten metal disposed above the column and from which the column is replenished, that improvement which consists in maintaining the head of the metal above the column below an approximate maximum depth of six inches throughout the casting process, whereby surface imperfections in the cast shape are avoided.

4. The process according to claim 3 characterized in that metal is added to the supply above the column without imparting turbulence to said column and while maintaining the movement thereof.

5. The process for casting copper and its alloys which comprises continuously supplying the metal to be cast to one end of a jacketed mold, continuously circulating a cooling fluid through said jacket at a rate sufficient to maintain the intermediate zone at a depth substantially no greater than the shortest cross-sectional dimension of the mold cavity and to solidify the metal with a predominantly radial crystal structure, and continuously withdrawing the fully solidified casting from the other end of said mold.

6. The process for casting nonferrous metals and alloys which comprises continuously supplying molten metal to a vertically disposed mold, continuously withdrawing solidified metal from said mold, and continuously extracting heat from the metal laterally to the direction of movement of the metal at a rate such that the intermediate zone between the metal in its molten and solidified states is constantly maintained at a depth not substantially greater than the diameter of the casting.

35 7. The process for casting aluminum which comprises continuously supplying molten aluminum to a vertically disposed mold, continuously withdrawing solidified aluminum from said mold, and continuously extracting heat from the aluminum laterally to the direction of movement of the aluminum at a rate such that the intermediate zone between the aluminum in its molten and solidified states is constantly maintained at a depth not substantially greater than the diameter of the casting.

8. In a process for casting copper and copper alloys in a continuous manner by laterally extracting heat from a moving, vertical column of the molten copper or copper alloy, the improvement which consists in so correlating the rates

of cooling and of movement of the column that the intermediate zone between the molten and solidified states of the copper or alloy is maintained at a depth not substantially greater than the diameter of the moving column.

9. In the process according to claim 8, the improvement that consists in continuously replenishing the metal of the column without turbulence thereto and while continuing its movement.

10. The process for continuously casting non-ferrous metals and alloys which comprises supplying the molten metal to the upper end of a vertically-disposed mold, extracting from the molten metal through the mold wall at least a part of the heat required to be dissipated for full solidification of the metal while maintaining the intermediate zone between the metal in its molten and fully solidified states wholly within the confines of the mold and at a depth not substantially greater than the minimum cross sectional dimension of the casting, and withdrawing the fully solidified casting out of the lower end of the mold.

11. The process for continuously casting copper and its alloys which comprises supplying the molten metal to the upper end of a vertically-disposed mold, continuously forming the molten metal into a fully solidified casting wholly within the confines of the mold by laterally cooling the same and while constantly maintaining the intermediate zone between the metal in its said fully molten and fully solidified states at a depth substantially no greater than the minimum cross sectional dimension of the casting, and withdrawing the fully solidified casting from the lower end of the mold.

12. The process for continuously casting non-ferrous metals and alloys which comprises confining the molten metal as a moving column, and transforming same into a moving column of fully solidified metal prior to emergence from confinement by extracting substantially all of both the superheat and the latent heat from the molten metal in a common path of heat flow transversely to the direction of movement of the column, the intermediate zone in the column being constantly maintained at a depth substantially no greater than the minimum cross sectional dimension of said column.

JESSE O. BETTERTON.  
FRANK F. POLAND.